

Nov. 19, 1929.

S. G. NYE

1,736,619

PROCESS OF TREATING GLASS FOR ILLUMINATION PURPOSES

Filed Feb. 14, 1928

Fig. 1.



Fig. 2.



Fig. 3.



Fig. 4.



Fig. 5.



Fig. 7.



Fig. 6.



*Inventor*  
**Sherman G. Nye**

*By John Smirle*

*Attorneys*

## UNITED STATES PATENT OFFICE

SHERMAN G. NYE, OF DENVER, COLORADO, ASSIGNOR, BY DIRECT AND MESNE ASSIGNMENTS, OF PART INTEREST TO OSCAR D. CASS AND E. E. NEWMAN, BOTH OF DENVER, COLORADO

## PROCESS OF TREATING GLASS FOR ILLUMINATION PURPOSES

Application filed February 14, 1928. Serial No. 254,317.

This invention relates to a process of treating the surface of glass closure plates for automobile lamps, or of lighting fixtures where glass is ordinarily used for the transmission of light from a source of intensive illumination.

The main object of the invention is to provide a process for treating the surface of the glass so as to eliminate the glare commonly produced by the transmission of light through clear untreated glass.

A further object of the invention is to treat the glass so as to obtain a very intense highly diffused light without objectionable sacrifice of illumination effect to obtain the desired diffusion.

Other objects of the invention will appear as the detailed description of the invention proceeds.

In order that the process of treating the glass may be clearly understood, reference is made to the accompanying drawings, in which:

Figure 1 is a perspective view of a circular disk of plain glass before being subjected to the process described herein;

Figure 2 is a plan view of the disk showing one face of the disk after being subjected to the first step in the process;

Figure 3 is similar view of the same face of the disk with an annular mat applied to said face before subjecting it to the second step in the process;

Figure 4 is a plan view of the disk after the second step of the process has been carried out on the previously treated face of the disk;

Figure 5 is a similar view of the treated face of the disk after completion of the second step, but with a second mat having a slightly larger circular opening substituted for the first mat;

Figure 6 is a plan of the finished disk; and

Figure 7 is a fragmentary section to an enlarged scale taken on the line 7-7 of Figure 6.

As shown in the several figures of the drawings, a sheet 1 of plain glass, preferably plate glass of good quality, is cut to the desired shape to adapt it for any particular use desired. In the present instance, it is cut to

form a circular disk adapted for use in an automobile headlight. The first step in the process of treating the disk consists in finely frosting one face of the disk 1 by any desired method—either by grinding or by sand-blasting it to produce the desired frosted effect.

Preferably the next step is to paste or otherwise secure an annular mat or stencil 2 to the frosted face. The radial width of the annulus between the peripheries of its inner and outer rings is preferably about one-fourth the diameter of the disk. The frosted face of the disk 1 within the circle 3 is then thoroughly impregnated with clear white vaseline or any clear transparent oil, rubbed into the frosted face inside the circle 3. The mat 2 is then removed, leaving the disk 1 with a circular area 4 coated with oil and with an annular area 2' frosted and dry.

The next step in the process consists in suitably fixing a mat or stencil 5, having its central circular opening 6 of slightly larger diameter than circle 3, to the frosted annular part 2' of the disk 1. The stencil 5 is arranged with its opening concentric with the oiled part 4 to leave an annular frosted space 7 between the periphery of circle 6 and the circular edge 8 of the oiled part. The oiled circle 4 and the frosted annulus 7 are then coated with a clear transparent lacquer which is allowed to dry.

Finally, the second mat 5 is removed and the finished disk is ready for use. As finished this disk comprises a sheet of glass having one face plain and its other face frosted, the frosted face having an outer annular part 9 uncoated and having a transparent lacquer skin 10 centrally secured to the frosted face to form therewith a cell having oil interposed between the lacquer skin and the frosted face of the glass.

While the lacquer is referred to as forming a skin over the oil, it must be understood that this is for purpose of description only. It is not known whether it mixes in some peculiar manner with the oil or not. It is known, however, by experimental use extending over a year that the lacquer coating does prevent spreading of the oil over the

frosted face of the disk, and may be freely rubbed by the hand without showing any trace of contact with the oil.

In addition to its intensity, the light emitted has no "glare" effect, and its uniform diffusions eliminates the shadows and zones of relative darkness so common with lenses having irregular diffracting surfaces.

The process must not be considered as limited in anyway to circular disks having only a partly oiled frosted surface. The whole frosted surface may be oiled; but the oiled frosted surface must also be lacquered. Neither oil nor lacquer alone will produce the desired result; nor will oil or lacquer, or lacquer and oil produce the desired effect on unfrosted glass. It is essential that the glass be plain on one side, frosted on the other; that the frosted side be wholly or partially coated with oil well rubbed in to the frosted glass; and finally that the oiled and frosted glass be covered with a transparent lacquer or the equivalent thereof.

What I claim is:

25 1. A lens for lamps comprising a sheet of glass having one face thereof plain and the other face roughened, a coating of transparent oil on the said other face, and a coating of transparent material superposed on the oil coating.

2. The process of treating plain transparent glass to form a lens for illumination purposes which consists in roughening one face of said glass, oiling part of said roughened face, and coating the oiled roughened surface with a transparent lacquer.

3. A lens for lamps comprising a circular disk of transparent plain glass having one face thereof frosted by roughening, a circular coating of oil of smaller diameter than said disk and concentrically arranged thereon, and a coating of transparent lacquer covering the oiled part of said disk.

In testimony whereof I affix my signature.

45 SHERMAN G. NYE.

50

55

60

65